

3,188,239

## SPINNERET CLEANING PROCESS

Heimen Kloppers, Leuvenheim, Netherlands, assignor to American Enka Corporation, Enka, N.C., a corporation of Delaware

No Drawing. Filed Feb. 4, 1963, Ser. No. 256,144  
Claims priority, application Netherlands, Feb. 16, 1962,  
274,929

9 Claims. (Cl. 134—26)

This invention relates generally to the cleaning of apparatus used in the melt extrusion of thermoplastic polymers and more particularly to a method for cleaning spinnerets that have become contaminated and clogged with the thermoplastic polymer and other substances during the production of synthetic filaments and yarn.

Various methods are known for cleaning spinnerets used in the melt spinning of such thermoplastic materials as polyamides, polyesters, polyurethanes, and polyolefins. In one method found fairly successful, they are cleaned by immersing the contaminated spinneret in a molten salt bath consisting of a mixture of alkali metal nitrate and alkali metal nitrite. In this process the temperature of the molten salt mixture ranges from 200–600° C. By using this cleaning method, deposits of the synthetic polymer or decomposition products thereof are converted into gaseous products or dislodged, thus leaving the spinneret surfaces clean.

However, recent developments in spinning procedures have rendered this cleaning method ineffective. In accordance with the present spinning practice, spinnerets are subjected during spinning to a treatment with liquid polyorganosiloxanes to guarantee that the spinning process may be carried on for an extended period without interruption. This material is usually intermittently sprayed onto the spinneret surface throughout the spinning operation. Polyorganosiloxanes useful for this purpose have the following formula:



wherein R is an alkyl group, aryl group, alkaryl group, or aralkyl group, and n is an integer greater than 1. Particularly preferred polysiloxanes for use in this treatment are the polymethylsiloxanes having a viscosity ranging from 500 to 1000 centistokes at 25° C.

Although the uninterrupted spinning time of spinnerets treated with polyorganosiloxanes is increased considerably, there are certain disadvantages to such a treatment. The high temperatures maintained during the melt spinning process cause a solid deposit to form on the spinneret surfaces which must be removed from time to time to insure satisfactory spinnability. In this connection, it has been found that the deposits, which originate from the polyorganosiloxanes, are not removed by the known molten salt bath spinneret cleaning method. Such a salt bath cleaning removes the polymer deposits but leaves polyorganosiloxane residues.

It is therefore an object of this invention to provide a method for cleaning spinnerets that have been treated with a polyorganosiloxane during the melt spinning of polymeric materials that does not have the disadvantages of the prior art spinneret cleaning method.

A further object of this invention is to provide a process for cleaning spinnerets that have been treated with a polyorganosiloxane during the melt spinning of polymeric materials that will remove not only contaminants and deposits originating with the polymeric material extruded, but will also remove the polyorganosiloxane and decomposition products thereof from the spinneret.

A still further object of this invention is to provide a spinneret cleaning method which is simple, efficient, and inexpensive, and that will not damage the spinneret.

These and other objects will be apparent from the following detailed description.

In accordance with this invention, it has been found that polyorganosiloxane deposits on the spinneret can be removed utilizing the known salt bath cleaning method if, prior to immersing the spinnerets in the alkali metal nitrate and nitrite bath, the spinneret is subjected to a pretreatment with white mineral oil. Such a pretreatment is easy to incorporate in the normal spinneret cleaning routine customarily used. In accordance with the invention, the contaminated spinnerets are either immersed in a white mineral oil such as a paraffin oil or simply smeared with the oil, and then soaked in a molten salt bath consisting of a mixture of alkali metal nitrate and alkali metal nitrite for a sufficient period of time to dislodge and decompose all foreign matter on the spinneret surfaces. Soaking time may range from 1/2 hour to 6 hours, depending on the degree of contamination. Upon withdrawal of the spinneret from the bath, all foreign deposits, including polyorganosiloxane contaminants, have been removed from the spinneret surfaces.

The purpose of the mineral oil in the inventive process is to provide a solvent action on the surface of the spinneret which aids the oxidation reaction carried out by the molten alkali salts. The only requirement as to the type of mineral oil used to produce this solvent effect during submersion into molten salt bath is that the hydrocarbon mineral oil must have a boiling point, i.e., vaporize, higher than the ambient temperature. This is necessary to enable the spinneret to be coated with the mineral oil when it is contacted by the molten salt bath.

For purposes of further illustration, the following examples are given. However, they are not to be construed as limiting the scope of the invention.

### Example I

A polyamide prepared from hexamethylene diamine and adipic acid was melt spun into filaments using two separate spinnerets. During the spinning process, each spinneret was from time to time sprayed with polymethylsiloxane. After the spinnerets had been used in this manner for two weeks, they were removed from the machine. One spinneret was immersed in a melt maintained at 450° C. containing about 50% by weight potassium nitrate and 50% by weight sodium nitrite for about 5 hours. The spinneret was thereafter cooled in air and washed with warm water to remove the salt. All polyamide contaminants previously adhering to the spinneret were removed by this treatment. However, the polymethylsiloxane deposits remained. The other spinneret after removal from the spinning machine was dipped in a white mineral oil bath, whose viscosity at 20° C. was about 35 centistokes, having a specific gravity of about .87. It was thereafter immersed in a 50% by weight potassium nitrate and 50% by weight sodium nitrite melt maintained at 450° C. for about 5 hours and then washed with warm water to remove traces of the salt. The spinneret was completely free from all polyamide and polymethylsiloxane deposits.

### Example II

A polyamide prepared from hexamethylenediamine and adipic acid was melt spun into filaments. Two spinnerets utilized in the spinning process were both sprayed with polymethylsiloxane throughout the spinning. After they had been used for about three weeks, they were removed from the spinning apparatus. One spinneret was immersed for about 5 hours in a melt containing 50% by

weight sodium nitrate and 50% by weight sodium nitrite maintained at about 500° C. The spinneret was cooled and rinsed with warm water. No trace of the polyamide remained on the spinneret. However, the polymethylsiloxane deposits were still present. The other spinneret was dipped in a white mineral oil bath identical with that of Example I, and then immersed for about 5 hours in the sodium nitrate, nitrite bath under the same conditions as the spinneret which had not received the mineral oil pretreatment. After it had been cooled and rinsed with warm water, it was found to be perfectly clean.

As the foregoing examples clearly indicate, the method of this invention cleans spinnerets in a practical and efficient manner without leaving any traces of polymer melt or polyorganosiloxane deposits.

It will be apparent to those skilled in the art that many widely different embodiments of this invention may be made without departing from the spirit and scope thereof, and therefore the invention is not intended to be limited except as indicated in the following claims.

What is claimed is:

1. A method for cleaning apparatus used in the melt extrusion of polymeric material, said apparatus having been coated with a polyorganosiloxane during the extrusion process, consisting essentially of coating said apparatus with a white mineral oil and thereafter immersing the apparatus in a molten salt bath consisting of a mixture of alkali metal nitrite and alkali metal nitrate for a sufficient period of time to dislodge and decompose all foreign matter on the spinneret surfaces.

2. The process of claim 1 in which the alkali metal salts are selected from the group consisting of potassium and sodium salts.

3. A method for cleaning spinnerets used in the melt extrusion of polymeric materials, said spinnerets being contaminated with the polymeric material extruded together with a polyorganosiloxane applied to the spinneret during the extrusion operation, having the formula:



wherein R is a member selected from the group consisting of alkyl, aryl alkaryl and aralkyl groups and n an integer greater than 1, consisting essentially of coating the spinnerets with a white mineral oil and thereafter immersing

them in a molten salt bath consisting of a mixture of alkali metal nitrite and alkali metal nitrate for a period of time sufficient to dislodge and decompose all foreign matter on the spinneret surfaces.

4. The method of claim 3 in which the alkali metal salts are selected from the group consisting of sodium and potassium salts.

5. A method for cleaning spinnerets used in the melt spinning of polymeric materials, said spinnerets being contaminated with the said polymeric material and polymethylsiloxane applied during the spinning operation consisting essentially of coating the spinneret with a paraffin oil and thereafter immersing the spinneret in a molten salt bath consisting of 50% by weight potassium nitrate and 50% by weight sodium nitrite for a sufficient period of time to dislodge and decompose all foreign matter on the spinneret surfaces.

6. The process of claim 5 in which the spinneret is immersed in the salt bath for about 5 hours.

20 7. The process of claim 1 in which the salt bath comprises a mixture of 50% by weight sodium nitrate and 50% by weight potassium nitrite.

8. The process of claim 5 in which the temperature of the molten salt bath is maintained at about 200-600° C.

25 9. A method for cleaning spinnerets used in the melt spinning of a polymeric material selected from the group consisting of polyamides, polyesters, polyurethanes and polyolefins, said spinneret being contaminated with said polymeric material together with polymethylsiloxane applied during the spinning operation, consisting essentially of coating the spinneret with a paraffin oil and thereafter immersing the spinneret for about 5 hours in a molten salt bath consisting of 50% by weight potassium nitrate and 50% by weight sodium nitrite, maintained at a temperature of about 450° C.

#### References Cited by the Examiner

#### UNITED STATES PATENTS

40 2,897,104 7/59 Duncan ----- 134-29

#### FOREIGN PATENTS

45 796,770 6/58 Great Britain.  
848,956 9/60 Great Britain.

DONALL H. SYLVESTER, Primary Examiner.